

1

3,751,363

**PIPE THREAD LUBRICANT STABILIZED WITH  
ORGANIC SULFIDES**

Raymond Rohde and Marvin M. Johnson, Bartlesville,  
Okla., assignors to Phillips Petroleum Company  
No Drawing. Filed Feb. 9, 1971, Ser. No. 114,042  
Int. Cl. C10m 5/16, 5/22

U.S. Cl. 252—19

6 Claims

**ABSTRACT OF THE DISCLOSURE**

Pipe thread lubricants comprising mineral oil, metal dust selected from lead, zinc, or alloys thereof, and alkaline earth metal soap and containing a stabilizing amount of an organic sulfide having the formula  $R-S_n-R'$  wherein  $R$  and  $R'$  are hydrocarbon radicals of 2 to 20 carbon atoms and  $n$  is an integer of from 2 to 4.

**BACKGROUND OF THE INVENTION**

This invention relates to pipe thread lubricants. In one of its aspects, it relates to antigalling thread lubricants containing metal particulate dust. In another of its aspects, it relates to stabilizing metal-dust-containing lubricants against reaction with water.

In one concept of the invention it relates to preventing the decomposition of a metal-dust-containing, antigalling thread lubricant by addition of a stabilizing compound to the lubricant to prevent reaction of the metal dust with water.

In the drilling of deep wells in the oil and gas industries high torque and elevated temperatures are encountered in the drilling operations which cause frequent problems of thread galling and joint seizure of the drill piping. The drill piping is expensive and its recovery and reuse is essential to an economic drilling operation. To increase the probability of recovery of the drill piping an antigalling thread lubricant is used. Most pipe thread lubricants include one or more powdered solids dispersed in various types of lubricating bases. The most advantageous of these lubricants are mixtures of metallic dust in high temperature alkaline earth metal-based grease, such as a mixture of zinc dust and a high temperature calcium-based grease.

Unfortunately exposure of a mixture of a metallic dust and a high temperature alkaline earth-based grease to moisture during storage can cause a reaction which produces explosive mixtures of hydrogen, i.e., zinc dust and water will react to produce hydrogen and zinc oxide. Ruptures of containers resulting from the gas accumulation during storage of this material have been reported repeatedly. Hydrogen gas explosions are also a possibility and both phenomena may have taken place simultaneously.

To avoid these hazards sulfur or nitrobenzene have been added to this type lubricant as stabilizers. While these stabilizers reduce the problem of hydrogen formation, other disadvantages have appeared. Nitrobenzene is a skin irritant continued exposure to which results in headaches and nausea. The amount of sulfur necessary to prevent hydrogen formation causes a chemical reaction with the grease to produce products which are corrosive to the drill pipe.

It is therefore an object of this invention to provide a metallic dust-containing, antigall thread lubricant stabilized against decomposition by reaction with water. It is another object of this invention to provide a stabilized antigall thread lubricant that is free of health hazards and metallurgical decomposition effects. It is another object of this invention to provide a means for stabilizing antigall thread lubricants.

2

Other aspects, concepts and objects of the invention are apparent from a study of this disclosure and the appended claims.

**SUMMARY OF THE INVENTION**

According to the present invention there is provided a stable antigall thread lubricant based on a lubricating composition of mineral oil, metallic dust, and an alkaline earth metal soap to which is added a stabilizing amount of an organic sulfide having a formula  $R-S_n-R'$  wherein  $R$  and  $R'$  are chosen from aliphatic and aromatic hydrocarbon radicals of 2 to 20 carbon atoms, not necessarily identical, and  $n$  is an integer of from 2 to 4.

In one embodiment of the invention dietary butyl disulfide is added as a stabilizer to a lubricant composition composed of mineral oil, zinc dust, and a calcium soap to stabilize the lubricant against decomposition by reaction with water.

The base grease compositions used in this invention are the metallic dust containing lubricants well known for use in the industry. These greases consist of a mineral oil or paraffin oil having a viscosity of 100 to 120 SUS at 210° F.; an alkaline earth metal soap, usually a calcium soap; and a metallic lubricating dust, usually lead, zinc or alloys thereof.

The mineral oil usually makes up from 25 to 75 percent by weight of the base grease composition. A preferred composition for the base grease contains from about 35 to about 55 percent by weight of mineral oil having a viscosity of 100 to 120 SUS at 210° F.

Any of the alkaline earth metal soaps can be used such as: alkaline earth metal salts of higher fatty acids having from 12-20 carbon atoms such as oleic, stearic, palmitic, myristic, linoleic, dodecanoic acids or mixtures thereof. Calcium stearate, calcium oleate, calcium palmitate, magnesium stearate, magnesium palmitate, strontium linoleate, barium dodecanoate, barium stearate, among others or mixtures of these may be used. The alkaline earth metal soap preferred in the composition of this invention is a calcium soap such as calcium stearate. Alkaline earth metal soap makes up from about 2 to about 10 percent by weight of the base grease composition and preferably is about 5 percent by weight of the base grease composition.

The metal dusts suitable for use in this invention include zinc, lead or alloys thereof, among others. Zinc is the preferred metal used as a lubricating metal dust in the composition of this invention. Powder of a particle size that will pass through a 200 mesh screen is advantageously used. The metal dust comprises from about 25 to about 75 percent by weight of the base grease composition and preferably will comprise in the range of about 40 to about 60 weight percent of the base grease composition.

The base grease composition is prepared by thoroughly blending the mineral oil, the metallic dust, and the alkaline earth metal soap. Such blends are well known in the art and any of the usual methods for obtaining a homogeneous blend of the ingredients may be used.

The inhibiting compounds useful in this composition are organic sulfides having the formula  $R-S_n-R'$  where  $R$  and  $R'$  are hydrocarbon radicals of 2 to 20 carbon atoms.  $R$  and  $R'$  can be the same or different and can be alkyl, aryl, or aryl-alkyl. The inhibitor compound can contain up to 4 sulfur atoms. Mixtures of sulfides can also be used. The inhibitor is added to the base grease formulation in amounts ranging from about 0.1 to about 5 parts per hundred parts of the formulated base grease. A preferred range for the inhibitor addition is about 0.2 to about 1.5 parts per hundred parts of formulated base grease. The compounds suitable for use in this invention are, among others,

|                                                                                 |    |
|---------------------------------------------------------------------------------|----|
| diethyl disulfide                                                               | 5  |
| di-n-propyl disulfide                                                           |    |
| di-tert-butyl disulfide                                                         |    |
| di-n-butyl disulfide                                                            |    |
| di-tert-hexyl disulfide                                                         |    |
| di-n-dodecyl disulfide                                                          |    |
| di-eicosyl disulfide                                                            |    |
| ethyl-tert-butyl disulfide                                                      |    |
| di-phenyl disulfide                                                             |    |
| tert-butyl hexyl polysulfide where $n$ has an average value between 2.5 and 3.5 | 10 |
| di-tert-dodecyl polysulfide where $n$ has an average value between 2.5 and 3.5  |    |
| di-tert-amyl polysulfide where $n$ has an average value between 2.5 and 3.5     | 15 |
| di-tert-butyl polysulfide where $n$ has an average value between 2.5 and 3.5.   |    |

The following are specific examples showing a test procedure for evaluating the inhibiting qualities of various additives for the composition of this invention and the effectiveness of selected additives as stabilizers for this composition.

#### EXAMPLE I

A base grease was prepared by thoroughly blending 40 parts by weight mineral oil having a viscosity of 100-120 SUS at 210° F., 55 parts by weight zinc dust and 5 parts by weight calcium soap to obtain a homogeneous mixture. To this base grease was added 0.5 percent by weight of the compounds to be tested as inhibitors. The test inhibitors, when added, were thoroughly blended into the composition. The inhibiting compounds tested are shown in Table I below.

#### EXAMPLE II

Approximately 25 grams of a lubricating compound of Example I was sealed in a 4-inch pressure tube; a 20 ml. hypodermic syringe inserted through the top; and the system (tube and syringe) flushed and blanketed with inert gas. The tube was immersed in a water bath at 140° F. The hypodermic syringe served as a gas expansion chamber. The tube remained in the water bath until gas evolution as measured by movement of the plunger was maximum. If no gas evolution occurred in two weeks the test was discontinued. If gas evolved it peaked in 5 to 7 days. The gas phase in the system consisting of inert blanket gas and generated gas was analyzed by gas chromatography to determine the amount of hydrogen that had been evolved.

The attached Table I summarizes the results obtained. Six tests were conducted on the base pipe thread compound (uninhibited)+1 percent water and no additive. Four of the six tests gave sizable evolution of hydrogen.

TABLE I.—GAS ANALYSIS

|                                          | Zinc dust drilling compound uninhibited plus 1% H <sub>2</sub> O | Gas evolved | Composition of gas phase in bottle (mol percent) |          | 55 |
|------------------------------------------|------------------------------------------------------------------|-------------|--------------------------------------------------|----------|----|
|                                          |                                                                  |             | Inert gas                                        | Hydrogen |    |
| No additive.....                         | None.....                                                        | None.....   | 99.5                                             | 0.5      |    |
| Do.....                                  | do.....                                                          | do.....     | 99.3                                             | 0.7      |    |
| Do.....                                  | Yes.....                                                         | 45.0        | 55.0                                             |          | 60 |
| Do.....                                  | Yes.....                                                         | 52.4        | 47.6                                             |          |    |
| Do.....                                  | Yes.....                                                         | 43.0        | 57.0                                             |          |    |
| Do.....                                  | Yes.....                                                         | 44.9        | 55.1                                             |          |    |
| Plus 0.5% nitrobenzene.....              | None.....                                                        | 99.6        | 0.4                                              |          |    |
| Do.....                                  | do.....                                                          | 99.6        | 0.4                                              |          |    |
| Plus 0.3% (zinc dithiophosphate).....    | Yes.....                                                         | 97.8        | 2.2                                              |          |    |
| Do.....                                  | Yes.....                                                         | 57.0        | 43.0                                             |          |    |
| Plus 0.5% quinone.....                   | None.....                                                        |             |                                                  |          |    |
| Do.....                                  | Yes.....                                                         | 76.3        | 22.4                                             |          |    |
| Plus 0.5% diteriary butyl disulfide..... | None.....                                                        | 99.2        | 0.8                                              |          |    |
| Do.....                                  | do.....                                                          | 99.4        | 0.6                                              |          |    |
| Do.....                                  | do.....                                                          |             |                                                  |          |    |
| Do.....                                  | do.....                                                          |             |                                                  |          |    |
| Do.....                                  | do.....                                                          |             |                                                  |          |    |

This table indicated that the production of hydrogen is quite likely when water is present with the uninhibited lubricating compound, and that, although hydrogen can be produced when a sulfide inhibitor is employed, the amount of hydrogen produced is not sufficient to be dangerous. This table also indicates the effectiveness of both nitrobenzene and diteriary butyl disulfide as inhibitors of the reaction of the zinc dust and water according to this invention. As noted before nitrobenzene has noxious qualities which make it undesirable as an additive in this type composition.

Reasonable variation and modification are possible within the scope of the foregoing disclosure, and the appended claims to the invention the essence of which is that organic sulfide compounds are effective stabilizers to prevent the reaction of metallic dust and water in anti-galling thread lubricants.

We claim:

1. A stable lubricating composition comprising (1) a formulated base grease of mineral oil vehicle, an effective amount of a metal dust selected from the group consisting of lead, zinc, or alloys thereof, and alkaline earth metal soap thickener and (2) a stabilizing amount of an organic sulfide having the formula R—S<sub>n</sub>—R' wherein R and R' are chosen from aliphatic and aromatic hydrocarbon radicals having 2 to 20 carbon atoms, not necessarily identical, and n is an integer of from 2 to 4.

2. The composition of claim 1 comprising about 0.1 to about 5 parts of organic sulfide per hundred parts of formulated base grease.

3. The composition of claim 1 wherein the formulated base grease is comprised of about 25 to about 75 percent by weight of a mineral oil having a viscosity of 100 to 120 SUS at 210° F., about 75 to about 25 percent by weight of a metal dust; and about 2 to about 10 percent by weight of an alkaline earth metal soap.

4. The composition of claim 3 wherein the metal dust is zinc, the alkaline earth metal soap is calcium soap, and the organic sulfide is diteriary butyl disulfide.

5. A method of inhibiting from reaction with water a lubricating formulation comprising a formulated base grease of mineral oil vehicle, an effective amount of a metal dust selected from the group consisting of lead, zinc, and alloys thereof, and alkaline earth metal soap thickener by incorporating therein a stabilizing amount of an organic sulfide having the formula R—S<sub>n</sub>—R', wherein R and R' are chosen from aliphatic and aromatic hydrocarbon radicals having 2 to 20 carbon atoms, not necessarily identical, and n is an integer of from 2 to 4.

6. The method of claim 5 wherein the organic sulfide is incorporated into the lubricating formulation in amounts in the range of about 0.1 to about 5 parts per hundred parts of lubricating formulation.

#### References Cited

#### UNITED STATES PATENTS

|           |         |                 |          |
|-----------|---------|-----------------|----------|
| 1,758,598 | 5/1930  | Fritzell        | 252—19   |
| 2,065,247 | 12/1936 | Smith           | 252—19   |
| 2,065,248 | 12/1936 | Smith           | 252—19   |
| 2,205,990 | 6/1940  | Nelson et al.   | 252—19   |
| 2,211,373 | 8/1940  | Folda           | 252—19   |
| 3,507,789 | 4/1970  | Heilweil et al. | 252—19   |
| 2,158,668 | 5/1939  | Rosen           | 252—46.4 |

DANIEL E. WYMAN, Primary Examiner

I. VAUGHN, Assistant Examiner

U.S. Cl. X.R.